

## ODOR STABILIZED LUBRICATING OIL ADDITIVES

John D. Bartleson, Beachwood Village, and Harvey E. Alford, Amherst, Ohio, assignors to The Standard Oil Company, Cleveland, Ohio, a corporation of Ohio

No Drawing. Application July 29, 1952,  
Serial No. 301,609

9 Claims. (Cl. 252—32.7)

This invention relates to an additive for lubricating oil to inhibit the deterioration thereof under service conditions, and which does not develop objectionable odors during use.

It has been proposed heretofore to react a phosphorus sulfide, such as phosphorus pentasulfide, with various hydrocarbons, including paraffins and cyclic aliphatics, for the purpose of producing a lubricating oil additive. The art recognizes that such reaction products are good additives, and in general their effectiveness can be measured, at least in part, by their sulfur content.

One of the inherent disadvantages of these additives is the development of hydrogen sulfide in an oil in which the additive has been incorporated. The objectionable odor of hydrogen sulfide renders these additives almost useless on a commercial scale for certain purposes, since the ordinary motorist will not tolerate such an odor in the oil at the time it is being added to the engine, or the development of such an odor during the use of the oil in the engines.

It is perhaps because of this inherent characteristic of such additives that the principal commercial additives are derived from organic compounds. The organic materials are relatively expensive as starting materials compared with hydrocarbon stocks. Furthermore, the manufacturers of lubricating oils are dependent upon the availability of such organic compounds from sources outside their manufacturing establishments. If a method could be developed in which the starting material for reaction with phosphorus sulfide is already available in an oil refinery, such as for instance a solvent-extracted lubricating oil, which method would provide an additive which was free from hydrogen sulfide or the development thereof, the refinery would have its own source of raw material for making a useful additive.

Accordingly, it is an object of our invention to develop a process of preparing an additive, and to provide the additive so prepared, utilizing a hydrocarbon stock as a starting material for reaction with a phosphorus sulfide, and the subsequent treatment thereof to eliminate hydrogen sulfide therefrom and eliminate the development of hydrogen sulfide in the oil containing the additive when the oil is used under service conditions.

These results are obtained by reacting an oil of lubricating viscosity with a phosphorus sulfide in proportions and under conditions to be described subsequently. This additive has satisfactory inhibitory properties, but contains hydrogen sulfide. Even though this be eliminated from the additive, such as by blowing the additive, it has been found that when the oil containing such a purified additive is heated at an elevated temperature, such as that developed in an internal combustion engine, hydrogen sulfide develops and can be detected when the engine is in use. In accordance with our invention, this objectional property is obviated by treating the oil with an alkali metal hydroxide, followed by treatment with sulfur dioxide, preferably in the presence of a small amount of water. We have established, as will be shown by data

to be presented subsequently, that the treatment with an alkali metal hydroxide itself is not adequate, nor is the treatment with sulfur dioxide adequate. However, the treatment with both of these materials gives an eminently satisfactory product, especially when the sulfur dioxide treatment is carried out in the presence of a small amount of water.

The oils that may be used as the starting material for the reaction product are those having a lubricating viscosity, such as 10 to 500 centistokes at 100° F. They may be acid-refined or refined by solvent extraction processes. Acid-treated oils tend to give a reaction product somewhat darker in color than the solvent-extracted oils, which is less attractive commercially but, nevertheless, possesses satisfactory inhibitory properties. Oils of high viscosity, such as SAE 70, are more difficult to handle in the reaction on account of their viscosity and are more difficult to filter. The higher viscosities also tend to give darker colored reaction products and are more apt to produce sludge, which must be filtered out. Oils having a low viscosity index, such as V. I. of 70, give a product with less hydrogen sulfide initially but, on the other hand, produce additives of darker color. A study of all of the various oils has indicated that a solvent-extracted oil having an SAE 10 viscosity and a viscosity index of at least about 95 was the optimum, considering color, ease of filtering, absence of sludge formation and other factors. It will be understood, however, that the reaction products made from all of these oils respond to the subsequent treatments which constitute our invention and that the oil will be selected depending largely upon availability, the importance of a light color and ease of handling in manufacture.

The sulfide may be any of those used in the art, such as the sesqui, the penta or heptasulfides. Phosphorus pentasulfide is readily available and it is used for this reason.

The reaction temperature between the oil and the phosphorus sulfide may be varied between about 250° and 450° F. A temperature of about 350° F. appears to be optimum for maximum sulfur content. Higher temperatures give additives with lower sulfur content and also give reaction products which are darker. The lower sulfur content of the product indicates a more complete reaction since there is a greater stability against the development of hydrogen sulfide. Although products prepared at a temperature of 300° to 350° F. evolve hydrogen sulfide more readily, this objection is overcome by the subsequent steps of our process, and the lighter products obtained at this temperature are generally preferred commercially. While any temperature can be used within the range, a temperature of 300° to 350° F. is preferred, depending somewhat upon the reaction time.

The lower the reaction temperature, the longer should be the reaction time to introduce the requisite amount of sulfur, as might be expected. Higher temperatures require shorter reaction times. Regardless of the reaction temperature, an increased reaction time darkens the additive. Increased reaction time also lowers the amount of hydrogen sulfide in the additive. The reaction time will be within a period of thirty minutes to ten hours, but for a reaction temperature of 300° F., four hours appears to be optimum, and at a temperature of 350° F. the reaction time can be shortened to two hours.

The amount of the phosphorus sulfide reacted is also a function to some extent of the reaction time and the reaction temperature. In general, the amount may vary from 1 to 10%. Increased amounts of phosphorus sulfide result in increased sulfur concentration in the additive, especially at higher reaction temperatures and longer times. At lower temperatures, the smaller increased sulfur content of the additive does not justify using larger

amounts of the phosphorus sulfide. The amount preferably is within the range from  $2\frac{1}{2}$  to 5%, and at an optimum temperature of  $300^{\circ}$  F. and a reaction period of four hours, 3.75% phosphorus pentasulfide gives a sufficiently high sulfur content in the additive to warrant not using more.

The reactions may be carried out in the manner conventional in the art using, if desired, an inert atmosphere, filtering the reaction product, blowing with air or an inert gas, and other recognized techniques of finishing the additive.

All of the additives prepared over the range of all of the variables described heretofore possess satisfactory inhibitory properties for lubricating oils, but all of them always developed hydrogen sulfide when stored in oil solution in the normal concentrations used in compounding of oils or when used under service conditions.

One method proposed for eliminating the hydrogen sulfide was to treat the additive with an adsorbent, such as activated clay. This lowered the hydrogen sulfide content and rendered it stable in storage at  $150^{\circ}$  F. up to forty hours. This stability, however, is not regarded as sufficient, since resistance to the development of hydrogen sulfide for a longer storage period is necessary to insure resistance to hydrogen sulfide development in

the additive is added to a lubricating oil at a concentration of 5% and the oil containing the additive in this concentration heated to  $150^{\circ}$  F., it is noted that  $H_2S$  develops in 16 hours. Thus this treatment does not stabilize the oil against the development of hydrogen sulfide for the requisite time. Similar conclusions are to be drawn from a comparison of the other samples.

An increase in the amount of potassium hydroxide improves the odor properties of the additive, but as the amount of potassium hydroxide is increased, the amount of sulfur in the additive is reduced. Further experimental work indicated that an amount of potassium hydroxide to eliminate the hydrogen sulfide odor completely would have lowered the sulfur content of the additive to a point of impotency. Consequently, the use of potassium hydroxide alone is unsatisfactory in preventing hydrogen sulfide formation in the additive.

It is known, of course, that sulfur dioxide reacts with hydrogen sulfide to form elemental sulfur and water, and it was thought that perhaps the treatment with sulfur dioxide would not only eliminate hydrogen sulfide from the additive but might modify the sulfur components that yield the hydrogen sulfide upon storage.

The results of treating the additive with sulfur dioxide are shown in Table II:

TABLE II

| Sample No. | Oil                  | Percent $P_2S_5$ | Reaction Time, hrs. | Reaction Temperature, $^{\circ}$ F. | Percent $SO_2$    | $SO_2$ Treatment Temp., $^{\circ}$ F. | Percent Water in $SO_2$ Treatment | Optical Density of Additive | $H_2S$ in Additive, p. p. m. | Percent Sulfur in Additive | Additive Conc. in Oil, percent | Hours <sup>1</sup> to $H_2S$ Formation in Oil at $150^{\circ}$ F. |
|------------|----------------------|------------------|---------------------|-------------------------------------|-------------------|---------------------------------------|-----------------------------------|-----------------------------|------------------------------|----------------------------|--------------------------------|-------------------------------------------------------------------|
| 8-----     | SAE 30, 95 V. I----- | 5                | 1                   | 400                                 | None <sup>2</sup> | 300 <sup>3</sup>                      | None                              | 980                         | 86.2                         | 2.84                       | 5                              | 16                                                                |
| 9-----     | SAE 30, 95 V. I----- | 5                | 1                   | 400                                 | 1.0               | 300                                   | None                              | 1,450                       | 84.6                         | ( <sup>4</sup> )           | 5                              | 16                                                                |
| 10-----    | SAE 30, 95 V. I----- | 5                | 1                   | 400                                 | 3.0               | 300                                   | None                              | 1,590                       | 16.2                         | 3.00                       | 5                              | 16                                                                |
| 11-----    | SAE 10, 95 V. I----- | 3.75             | 4                   | 300                                 | None              | 225 <sup>4</sup>                      | 0.25                              | 133                         | 445.9                        | 2.03                       | 7.5                            | 16                                                                |
| 12-----    | SAE 10, 95 V. I----- | 3.75             | 4                   | 300                                 | 1.0               | 225                                   | 164                               | 61.5                        | 2.27                         | 7.5                        | 7.5                            | 16                                                                |

<sup>1</sup> 72 hours needed to pass this test.

<sup>2</sup> Treated at atmospheric pressure.

<sup>3</sup> Not measured.

<sup>4</sup> Treated at pressure of 5 p. s. i. g.

use. In addition, the treatment with such adsorbents not only did not solve the odor problem, but the sulfur loss of the additive was unusually high.

Inasmuch as it has been proposed heretofore to neutralize such reaction products with a base, such as potassium hydroxide, the treatment of the additives with flake KOH was attempted. This caustic potash is in the form of dry appearing solid flakes, although it contains about 15% water. The amount of KOH referred to herein is the amount in flake form. The results are shown in Table I, which follows:

45 A comparison of Samples 8, 9 and 10 shows that the sulfur dioxide treatment darkens the oil but reduces the hydrogen sulfide content of the additive. The amount of sulfur is also increased, as might be expected. A comparison of Samples 11 and 12 shows similar results. In the last sample, a small amount of water was added before the sulfur dioxide treatment, as indicated. When 50 all of these additives were incorporated in a lubricating oil at a concentration of 5%, the oil developed an odor of hydrogen sulfide within 16 hours after storage at  $150^{\circ}$  F. The use of pressure as indicated in Sample 12

TABLE I

| Sample No. | Oil                  | Percent $P_2S_5$ | Reaction Time, hours | Reaction Temperature, $^{\circ}$ F. | Percent KOH <sup>2</sup> | Optical Density of Additive | $H_2S$ in Additive, p. p. m. | Percent Sulfur in Additive | Additive Concentration in Oil, percent | Hours <sup>1</sup> to $H_2S$ Formation in Oil at $150^{\circ}$ F. |
|------------|----------------------|------------------|----------------------|-------------------------------------|--------------------------|-----------------------------|------------------------------|----------------------------|----------------------------------------|-------------------------------------------------------------------|
| 1-----     | SAE 30, 95 V. I----- | 5                | 1                    | 400                                 | None                     | 980                         | 86.2                         | 2.84                       | 5                                      | 16                                                                |
| 2-----     | SAE 30, 95 V. I----- | 5                | 1                    | 400                                 | 1                        | 865                         | 38.2                         | ( <sup>3</sup> )           | 5                                      | 16                                                                |
| 3-----     | SAE 30, 95 V. I----- | 5                | 1                    | 400                                 | 3                        | 780                         | 7.8                          | 1.47                       | 5                                      | 16                                                                |
| 4-----     | SAE 10, 95 V. I----- | 5                | 4                    | 300                                 | None                     | 298                         | 152                          | 2.42                       | 5                                      | 16                                                                |
| 5-----     | SAE 10, 95 V. I----- | 5                | 4                    | 300                                 | 0.9                      | 220                         | ( <sup>4</sup> )             | ( <sup>4</sup> )           | 5                                      | 16                                                                |
| 6-----     | SAE 30, 95 V. I----- | 2.5              | 1                    | 400                                 | None                     | 449                         | 26.2                         | 1.15                       | 10                                     | 16                                                                |
| 7-----     | SAE 30, 95 V. I----- | 2.5              | 1                    | 400                                 | 0.6                      | 378                         | 3.8                          | 0.89                       | 10                                     | 40                                                                |

<sup>1</sup> 72 hours required to pass this test.

<sup>2</sup> Not measured.

<sup>3</sup> Reacted at  $250^{\circ}$  F. for one hour.

A comparison of Sample No. 1 with Samples 2 and 3 shows that the use of KOH reduced the optical density, indicating a lighter color, and also reduced the amount of hydrogen sulfide in the additive. It is also be noted by a comparison of Samples 1 and 3 that the amount of sulfur in the additive is reduced by this treatment. When

70 does not appear to affect the result, nor did the presence of water affect the result. In the absence of any improvement whatever in odor stability, the use of sulfur dioxide by itself is impractical.

In accordance with our invention, we have discovered 75 that the combined steps of treating the additive with po-

tassium hydroxide and sulfur dioxide, especially in the presence of water, markedly improves the additive and gives it unusual storage stability properties.

The potassium hydroxide, preferably in the flake form described heretofore, is reacted with the additive at a temperature of 150 to 400° F. for from one-half to five hours. Higher temperatures require shorter reaction times. Any temperature or time which will result in the potassium hydroxide becoming absorbed is satisfactory. The amount of potassium hydroxide may vary from 0.25 to 5.0% based on the amount of the additive.

The amount of the sulfur dioxide reacted should be sufficient to give the requisite stability. This may vary with the additive, the materials from which it is made and the reaction conditions under which it is made. With the optimum form of additive, the minimum amount of sulfur dioxide is about 1.9%. The pressure of the sulfur dioxide reaction, the time and temperature of the sulfur dioxide reaction are all immaterial as long as the requisite amount of sulfur dioxide is absorbed and reacted. Generally, the pressure will be from atmospheric to about 50 lbs. per square inch gauge, and a reaction temperature of 150 to 250° F. will require a reaction time of about 4 hours to 1/2 hour. There appears to be no maximum amount of sulfur dioxide to be reacted because there is a limit to the amount that can react under given conditions.

It appears to be desirable to have a small amount of water, generally 0.25 to 1.0%, present during the sulfur dioxide reaction to activate this reaction, although this is not essential if a longer reaction time or otherwise vigorous reaction conditions are selected.

The results showing several optimum embodiments of the invention are given in Table III.

TABLE III

| Sample No. | Oil              | Percent P <sub>2</sub> S <sub>5</sub> | Reaction Time, hrs. | Reaction Temp., ° F. | Percent KOH <sup>4</sup> | Percent SO <sub>2</sub> | SO <sub>2</sub> Treatment Temp., ° F. | Percent Water in SO <sub>2</sub> Treatment | Optical Density of Additive | H <sub>2</sub> S in Additive, p. p. m. | Percent Sulfur in Additive | Additive Conc. in Oil, percent | Hours <sup>1</sup> to H <sub>2</sub> S Formation in Oil at 150° F. |
|------------|------------------|---------------------------------------|---------------------|----------------------|--------------------------|-------------------------|---------------------------------------|--------------------------------------------|-----------------------------|----------------------------------------|----------------------------|--------------------------------|--------------------------------------------------------------------|
| 13         | SAE 10, 95 V. I. | 3.75                                  | 4                   | 300                  | None                     | None                    | 275                                   | 0.25                                       | 100                         | 128.2                                  | 2.03                       | 7.5                            | 16                                                                 |
| 14         | SAE 10, 95 V. I. | 3.75                                  | 4                   | 300                  | 1.0                      | 2.2                     | 325                                   | 0.25                                       | 332                         | 1.83                                   | 7.5                        | 720                            |                                                                    |
| 15         | SAE 10, 95 V. I. | 3.75                                  | 4                   | 300                  | 1.0                      | 2.192                   | 225                                   | 0.25                                       | 170                         | 4.4                                    | 1.73                       | 7.5                            | 720                                                                |
| 16         | SAE 10, 95 V. I. | 3.75                                  | 4                   | 300                  | 1.0                      | 2.63                    | 250                                   | 0.25                                       | 166                         | 6.7                                    | 1.77                       | 7.5                            | 500                                                                |
| 17         | SAE 10, 95 V. I. | 3.75                                  | 4                   | 200                  | None                     | None                    | 225                                   | 0.25                                       | 112                         | 180.7                                  | 1.99                       | 7.5                            | 16                                                                 |
| 18         | SAE 10, 95 V. I. | 3.75                                  | 4                   | 300                  | 1.0                      | 2.16                    | 225                                   | 0.25                                       | 154                         | 14.3                                   | 2.01                       | 7.5                            | 500                                                                |
| 19         | SAE 10, 95 V. I. | 3.75                                  | 4                   | 300                  | 1.0                      | 2.16                    | 225                                   | 0.25                                       | 154                         | 14.3                                   | 2.01                       | 7.5                            | 4 500                                                              |

<sup>1</sup> 72 hours needed to pass test.

<sup>2</sup> Reacted at 5 p. s. i. g.

<sup>3</sup> Reacted at 10 p. s. i. g.

<sup>4</sup> 1% water added before tested and tested at room temperature.

<sup>5</sup> Reacted at 250° F. for one hour.

The above data clearly establish that the process of the invention overcomes the problem of hydrogen sulfide generation on storage. In addition, it does not interfere with the use properties of the additives under service conditions. As has already been indicated, the additive with its objectionable odor is a satisfactory inhibitor. As indicative of this, an additive was prepared employing the optimum conditions, namely, SAE 10 solvent-extracted oil having a viscosity index of 95, reacted with 3.75% phosphorus sulfide for four hours at 300° F. This additive was incorporated in the amount of 8% in an SAE 20 oil and the oil tested for 36 hours in the L-4 Chevrolet engine test. The results are shown in Table IV in the column headed "Untreated." The same additive treated in accordance with the invention, more particularly, in 1% KOH, 0.25% water and 2.14% sulfur dioxide, was incorporated in the same amount in the same base oil and subjected to the same tests. The results are shown in Table IV, under the column marked "Treated."

6  
TABLE IV  
Test: L-4 Chevrolet—36 hours

|                        | Additive | Treated | Untreated |
|------------------------|----------|---------|-----------|
| Piston Skirt           |          | 7.50    | 7.0       |
| Varnish (Total)        |          | 42.75   | 43.25     |
| Sludge (Total)         |          | 44.00   | 44.25     |
| Corrosion (gms.)       |          | 0.2898  | 0.1678    |
| Sohio Dermerit Rating: |          |         |           |
| Piston Skirt           |          | 2.5     | 3.0       |
| Sludge                 |          | 1.2     | 1.15      |
| Corrosion              |          | 2.9     | 1.7       |
| Used Oil               |          | 0.85    | 0.86      |
| Total Demerits         |          | 7.45    | 6.71      |

From the data in the above table, it is apparent that the additive prepared in accordance with the invention is substantially as good as the untreated additive, in addition to having the very desirable property of odor stability under service conditions.

The additive may be used in any concentration to give the requisite inhibiting action depending somewhat on the properties of the base oil and the amount of inhibition. Generally the additive will be in a minor amount such as 1 to 25%, preferably about 4 to 12%. Because the additive is inexpensive and utilizes readily available and inexpensive raw materials, it can be used in larger quantities than the more expensive additives. In order to determine the effectiveness in economic terms, the additive was tested and compared with a large number of additives commercially available on the market. These were all tested in the Polyveriform test as described in "Analytic Chemistry," 21, 737 (1949). The results are as follows:

TABLE V

|                                             | Amount of Additive Used, Percent | Cost in Cents/Gallon of Oil | Result in Percent of Perfect | Cost of Inhibitor Per 10% of Improvement in Cents |
|---------------------------------------------|----------------------------------|-----------------------------|------------------------------|---------------------------------------------------|
| Additive of the Invention                   | 8.3                              | 0.88                        | 60                           | 0.14                                              |
| 19 Other Commercial Additives on the Market | 1 to 8                           | 1.73 to 18.2                | 62 to 89                     | 0.265 to 2.15                                     |

From the above, it will be seen that although a relatively larger amount of the additive is used the cost in terms of the improvement is less than any other additives on the market which were tested.

We claim:

1. A method of preparing an additive which comprises reacting a mineral oil of lubricating viscosity with from 2 to 10% phosphorus sulfide at a temperature of

250 to 450° F. for from one-half to ten hours to form a lubricating oil additive, treating the additive with an alkali metal hydroxide followed by treatment with sulfur dioxide to provide an additive resistant to the development of hydrogen sulfide.

2. A method of preparing an additive which comprises reacting a mineral oil of lubricating viscosity with from 2 to 10% phosphorus sulfide at a temperature of 250 to 450° F. for from one-half to ten hours to form a lubricating oil additive, and treating the additive with from 0.25 to 5.0% flake potassium hydroxide containing a small amount of water for one-half to five hours at 150 to 400° F., followed by treatment with sulfur dioxide in the presence of a small amount of water to absorb at least about 1.9% sulfur dioxide by weight, to provide an additive resistant to the development of hydrogen sulfide.

3. A method of preparing an additive which comprises reacting an SAE 10 solvent-extracted lubricating oil with about 3.75% phosphorus pentasulfide at a temperature of about 300° F. for about four hours to form a lubricating oil additive, treating the additive with about 1% potassium hydroxide in flake form containing about 15% water for about one hour at about 250° F. followed by treatment with sulfur dioxide under pressure in the presence of about 0.25% water to absorb at least about 1.9% sulfur dioxide by weight, to provide an additive resistant to the development of hydrogen sulfide.

4. The lubricating oil additive made by the process of claim 1.

5. The lubricating oil additive made by the process of claim 2.

6. The lubricating oil additive made by the process of claim 3.

7. A lubricating oil comprising a major proportion of a mineral oil of lubricating viscosity and a minor amount to inhibit the deterioration of the oil under service conditions of an additive of claim 4.

8. A lubricating oil comprising a major proportion of a mineral oil of lubricating viscosity and a minor amount to inhibit the deterioration of the oil under service conditions of an additive of claim 5.

9. A lubricating oil comprising a major proportion of a mineral oil of lubricating viscosity and a minor amount to inhibit the deterioration of the oil under service conditions of an additive of claim 6.

References Cited in the file of this patent

UNITED STATES PATENTS

|    |           |                     |               |
|----|-----------|---------------------|---------------|
| 20 | 2,179,711 | Luten et al. -----  | Apr. 14, 1942 |
|    | 2,316,091 | White -----         | Apr. 6, 1943  |
|    | 2,367,468 | Mixon et al. -----  | Jan. 16, 1945 |
|    | 2,496,508 | Watson et al. ----- | Feb. 7, 1950  |
| 25 | 2,498,201 | Daigle -----        | Feb. 21, 1950 |
|    | 2,560,546 | Bartleson -----     | July 17, 1951 |
|    | 2,560,548 | Bartleson -----     | July 17, 1951 |
|    | 2,637,722 | Frazier -----       | May 5, 1953   |